

June 15, 1937.

S. M. SECRIST

2,084,298

METHOD OF LINING METALLIC VESSELS

Filed Nov. 8, 1934

*Fig. 1.*



*Fig. 2.*



*Fig. 3.*



*Fig. 4.*



*Fig. 5.*



*Inventor:*

STANLEY M. SECRIST,  
by *Asina & Chamber*  
*his Attorneys.*

## UNITED STATES PATENT OFFICE

2,084,298

## METHOD OF LINING METALLIC VESSELS

Stanley M. Sechrist, New York, N. Y., assignor to  
 American Sheet and Tin Plate Company, a  
 corporation of New Jersey

Application November 8, 1934, Serial No. 752,156

2 Claims. (CL 29—162)

This invention relates to an improved method of lining metallic vessels, and more particularly to the application of heat-and-corrosion resistant metallic linings (such as are composed of stainless steel) to metallic tanks, although not limited thereto.

It is among the objects of the present invention to provide a novel method of lining metallic vessels which may be rapidly and economically utilized under the most difficult and confining circumstances.

Another object is to enable the installation of high quality linings in tanks or vessels which might otherwise be discarded or become useless for certain purposes.

These and other objects will be apparent after referring to the drawing, in which:

Figure 1 is a sectional view of the medium to be treated in accordance with the method of the invention.

Figure 2 is a similar view of the medium of Figure 1 after the completion of the first stage.

Figure 3 is a similar view disclosing a third stage of the method.

Figure 4 graphically represents the combination of the novel method.

Figure 5 is a view similar to Figure 4 but representing the slight modification of the method.

Referring more particularly to the drawing, the numeral 10 designates a heavy metallic base, such as the inner side of a tank or vessel, for which there is desired a lining of high quality material. As an example, tanks formed of heavy steel plate, whose initial linings of glass, lead or the like have been found faulty and removed, may be reconditioned by substituting a high quality metal, such as stainless steel.

According to the teaching of the present invention, the metallic base 10, having sides 12 and 13, is apertured at spaced intervals, as shown at 14. As shown in Figure 2, these apertures 14 are preferably countersunk in such manner as to have their smallest openings 15 communicating with the side of the metallic base 10 for which the lining is desired (that designated at 13 in the present instance). The welding will be accomplished through the largest openings 16 of the apertures 14.

The lining for the side 13 of the metallic base 10 is shown in Figure 3 as comprising a relatively thin sheet of heat-and-corrosion resistant metal 17 which is placed over the smallest openings 15 of the apertures 14.

The next step in the method is to make evident on the exposed side of the lining 17 the loca-

tions of the apertures 14 with respect thereto. This may be done with a punch 18 which is applied through the apertures, as shown in Figure 3, and struck with a hammer (not shown); or as an alternative, the application of heat by arc or gas torch 19, as shown in Figure 4, in such manner as to discolor the exposed side of the lining 17.

After the locations of the apertures 14 are indicated on the exposed side of the lining 17 a heat conductive element 20 is placed thereover immediately prior to the welding per se. This heat conductive element 20, as shown in Figure 4, is preferably a copper ball mounted on a rod 21, and should be firmly held against the exposed side 15 of the lining 17. This may be done by a jack (not shown) in contact with the opposite side of the tank or vessel 10. Experiment has shown that the pressure exerted on the heat conductive element 20 should preferably be of sufficient magnitude to slightly distort the lining 17. This condition, as illustrated in dotted lines at 22 in Figure 5, not only secures a better contact for the effective dissipation of heat but also prevents the excessive discoloration of the exposed side 25 of the lining 17 by the spreading thereof.

A welding medium 23, preferably a filler metal of the same analysis as that of the lining 17, is introduced into the largest opening 16 of the aperture 14. This welding medium 23 forms a 30 rigid union between the metallic lining 17 and the metallic base 10, which under most circumstances would be of a dissimilar analysis. After sufficient welding medium 23 has been introduced into the aperture 14 to form a rigid union, it may be more or less completely filled with any suitable fusible metal 24, such as steel.

After the welding has been completed the metallic lining 17 will be found to serve satisfactorily under all conditions of usage, whether 40 stationary or movable.

While I have shown and described one specific embodiment of my invention, it will be understood that I do not wish to be limited exactly thereto, since various modifications may be made without departing from the scope of my invention, as defined in the following claims.

I claim:

1. The method of lining a metallic vessel which includes the operations of forming a plurality of apertures in said vessel, disposing a relatively thin imperforate sheet against the inner wall of the body of the metallic vessel, said thin imperforate sheet being composed of a metal which is dissimilar to that of said vessel, applying suc- 50 55

cessively and under pressure a heat conductive element to said thin imperforate sheet on its side remote from but in alignment with the plurality of apertures in said vessel, and securing said thin imperforate sheet to the inner wall of the body of the metallic vessel solely by forming weld plugs which are connected to the side walls of the apertures in said vessel and to the adjacent surface of said thin imperforate sheet, the formation 10 of each of said weld plugs being conducted from the outside of said vessel while said heat conductive element is in alignment with the particular aperture in which it is to be formed.

2. The method of lining a metallic vessel which includes the steps of forming an aperture in said vessel, disposing a metallic sheet against the inner wall of said vessel, deforming an unbroken surface of said sheet partially into the aperture 5 into said vessel, and welding the deformed and unbroken surface of said sheet to the wall of the aperture in said vessel, thereby affixing said sheet to the inner wall of said vessel, said welding step being carried out from outside of said vessel. 10

STANLEY M. SECRIST.